

# United States Patent

[19]

Suzuki et al.

4,004,406

[11] [45] Jan. 25, 1977

[54] SPUN TYPE YARN AND PROCESS FOR  
MANUFACTURING THE SAME

[75] Inventors: Hirotsugu Suzuki; Yo Ogawa;  
Yoshikazu Kikuchi; Shin-ichi  
Kitazawa, all of Otsu, Japan

[73] Assignee: Toray Industries, Inc., Tokyo, Japan

[22] Filed: Apr. 16, 1975

[21] Appl. No.: 568,654

[30] Foreign Application Priority Data

Apr. 22, 1974 Japan ..... 49-44497  
Feb. 3, 1975 Japan ..... 50-13358

[52] U.S. Cl. ..... 57/140 R; 57/157 R

[51] Int. Cl.<sup>2</sup> ..... D02G 3/02; D02G 3/26

[58] Field of Search ..... 57/140 R, 144, 157 R,  
57/157 MS, 157 F, 160, 34 R, 34 HS, 157 BY

## [56] References Cited

### UNITED STATES PATENTS

2,289,568 7/1942 Bloch ..... 57/140 R X

|           |         |               |       |             |
|-----------|---------|---------------|-------|-------------|
| 3,043,088 | 7/1962  | Breen         | ..... | 57/140 R X  |
| 3,111,805 | 11/1963 | Boyer         | ..... | 57/140 BY   |
| 3,538,701 | 11/1970 | Cannon et al. | ..... | 57/157 F    |
| 3,596,458 | 8/1971  | Nakano et al. | ..... | 57/140 BY X |
| 3,732,684 | 5/1973  | Csok et al.   | ..... | 57/157 F X  |

Primary Examiner—Donald E. Watkins

## [57] ABSTRACT

A spun-type yarn having a unique configuration and useful properties is manufactured by a novel process which comprises forming a ribbon-shaped fiber bundle being substantially free from twists and composed of randomly oriented continuous filaments, each of which comprises random bends and loops along its length, and then false twisting the ribbon-shaped bundle to consolidate it into a yarn. In the false-twisting, some of the filaments are broken.

16 Claims, 11 Drawing Figures



Fig. 1



Fig. 2



Fig. 3



Fig. 4



Fig. 5



Fig. 6



Fig. 7



Fig. 8



Fig. 9



Fig. 10



Fig. 11



## SPUN TYPE YARN AND PROCESS FOR MANUFACTURING THE SAME

This invention relates to a novel spun-type yarn having a unique configuration and a process for the manufacture thereof. More particularly, this invention relates to a novel spun-type yarn of a unique diversiform configuration and having useful properties and a false-twisting type process for manufacturing the same from a continuous filamentary fiber bundle.

### BACKGROUND OF THE INVENTION

In general, conventional ring spinning requires a number of preparatory steps in the manufacturing of spun yarns of synthetic fibers. Disadvantages of the conventional process are low productivity, nep formation and increasing irregularity in weight per length in the opening and drafting stages. Therefore, the conventional ring spinning requires redundant steps in addition to the indispensable steps. Further, even the complicated steps of the conventional process, it is very difficult to form fibers of poor physical properties, such as fibers of cured novolac resin or cured novolacpolyamide resin, into yarns. In manufacturing spun yarns of textile fibers, for example, polyester fibers, polyamide fibers and polyacrylic fibers, conventional ring spinning requires a restriction on the diameter of supplied staple fiber. Thus, it is very difficult to manufacture spun yarns made of fibers of fine denier.

Much research effort has been directed and many methods have been proposed to remove these defects of the conventional ring spinning, as shown in U.S. Pat. No. 3,079,746, U.S. Pat. No. 3,365,872 and British Pat. No. 1,102,095.

U.S. Pat. Nos. 3,079,746 and 3,365,872 disclose the manufacture of spun yarns made of discontinuous fibers or a combination of discontinuous fibers with continuous strands. However, since these patents are confined to only improvements in the twisting step, many of the preparatory steps for making slivers in the ring spinning process still need to be improved.

British Pat. No. 1,102,095 discloses a product and a process wherein some qualities characteristic of a spun staple fiber yarn are imparted to continuous filamentary yarn. Such yarns are apt to have many long radially-projecting loops. However, the presence of these radially-projecting loops, particularly the presence of long loops on the surface of the yarns, imparts undesirable properties to the yarn. For instance, in knitting fabrics, long loops induce irregular tension when the yarn is unwound from a cone or a bobbin and cause many defects in the fabrics.

### SUMMARY OF THE INVENTION

It is an object of this invention to prepare a spun-type yarn in various novel and useful forms.

Another object of this invention is to provide a novel and efficient process for manufacturing a spun-type yarn.

Other objects will become apparent from the following description as well as the accompanying drawings, and claims.

The novel spun-type yarn of this invention consists of a fiber bundle which is substantially free from true twists and composed of continuous and discontinuous filaments being complexly intertwined with one another and comprising random bends and loops along

their lengths. The yarn has a spun yarn-like hand and appearance and desirable properties for knitted and woven fabrics.

The above-mentioned yarn having a unique diversiform configuration and useful properties can be manufactured by a process which comprises forming a ribbon-shaped fiber bundle being substantially free from twists and having randomly oriented or arranged continuous filaments, each of which comprises random bends and loops along its length, and then false twisting said ribbon-shaped bundle to consolidate it into a yarn while some of the filaments are broken in the false twisting.

### BRIEF EXPLANATION OF THE DRAWINGS

FIG. 1 is an enlarged schematic illustration of a yarn of this invention;

FIG. 2 is a side view schematically illustrating one form of the apparatus for use in the process of this invention;

FIG. 3 is a perspective view schematically illustrating another form of the apparatus for use in the process of this invention;

FIG. 4 is an enlarged longitudinal cross-sectional view of one form of ejector useful in practicing this invention;

FIG. 5 is an enlarged longitudinal cross-sectional view of another form of ejector useful in practicing this invention;

FIG. 6 is an enlarged longitudinal cross-section view of one form of false-twisting device useful in practicing this invention;

FIG. 7 is an enlarged transverse cross-section view of the device shown in FIG. 6, taken on line X-Y of FIG.

35 6;

FIGS. 8 and 9 are examples of the staple diagram characteristic of the yarn of this invention, and;

FIGS. 10 and 11 represent the staple diagrams inherent to the yarns of prior arts.

### DETAILED EXPLANATION OF THE INVENTION

This invention provides a novel and useful spun-type yarn. In general, the yarn of the present invention consists of a fiber bundle which is substantially free from true twists and is composed of continuous and discontinuous filaments. These continuous and discontinuous filaments are complexly intertwined with one another and comprises random bends and loops along their lengths.

Referring now to FIG. 1, a typical yarn of this invention is schematically shown in an enlarged illustration. Some of the fiber bundle composing filaments are partially and randomly wrapped around the fiber bundle, while being intertwined with one another. The surface wrapping and entanglement as well as the entanglement within the fiber bundle give moderate coherency and strength to the yarn. Further, the yarn contains multiple free ends of broken, bent and looped filaments, which protrude from the fiber bundle of the yarn, so that the yarn possesses a spun yarn-like hand and appearance and, thus, can be made into fabrics having desirable functional properties such as those of spun yarn fabrics. The discontinuous broken filaments have irregular lengths and the surface wrapping filaments are wound around the fiber bundle at various angles with respect to the longitudinal axis of the yarn.

The above-mentioned unique and diversiform configuration of the yarn of the present invention may be

conveniently characterized by parameters S and R as described below.

A test piece is arbitrarily cut at a length of 10 mm along the length of a yarn under a load of 500 mg/denier and the fiber length of the respective fibers contained in the test piece is then measured. Next, the parameters S and R are defined as follows:

$$S = B/A$$

$$R = C/D$$

wherein A is the number of fibers whose length is in the range of not less than 10 mm but less than 12 mm, B is the number of fibers whose length is in the range of not less than 12 mm but less than 30 mm, C is the number of fibers whose length is not less than 30 mm and D is the number of fibers contained in the test piece.

Thus, the yarn of this invention preferably has a value of the parameter S of not less than 0.5, more preferably of not less than 1.0, and most preferably a value of the parameter S of not less than 1.0 and a value of the parameter R of not more than 0.1.

The properties represented by the parameters S and R will become apparent from the following explanation. In the case of yarns composed of multifilaments arranged parallel to the longitudinal axis of the yarn, the value of the parameter S is equal to zero. In a staple spun yarn obtained by conventional ring spinning, fibers are oriented or arranged in the lengthwise direction of the yarn by the drafting operation during the yarn manufacturing process. However, the value of the parameter S is not usually equal to zero because the yarn is actually twisted. In the case of a yarn which has many radially projecting short loops, radially projecting short fibers and/or wrapping fibers on the yarn surface, the value of the parameter S is fairly large and, in general, the yarn has desirable properties in bulkiness and uniformity of unwinding tension when the yarn is unwound from a cone or a bobbin.

As mentioned above, it is easily understood that the parameter S indicates the degree of orientation or arrangement of the yarn composing fibers and the properties, such as bulkiness and uniformity of unwinding tension, of the yarn. Parameter R is another measure of the uniformity of unwinding tension. A yarn of the parameter R having a large value is inferior in its uniformity of unwinding tension because of the presence of many radially projecting long loops and/or radially projecting long fibers on the yarn surface. From our experience, it has been confirmed that a yarn of the parameter S of not less than 0.5 and the parameter R of not more than 0.1 has the most desirable bulkiness and uniformity of unwinding tension.

The yarn of this invention is manufactured by the following novel process which comprises forming a ribbon-shaped fiber bundle being substantially free from twists and composed of randomly oriented or arranged continuous filaments, each of which comprises random bends and loops along its length, and then false twisting the ribbon-shaped bundle to consolidate it into a yarn. In the false-twisting operation, some of the filaments are broken by a means for false twisting.

The ribbon-shaped bundle may be formed by extruding polymer melt into filaments through a spinneret, stretching the filaments thus formed preferably pneumatically by compressed air jets and then depositing

them on a receiving conveyor which advances the filaments deposited thereon.

Referring to FIGS. 2 and 3 wherein similar parts are designated by the same reference numerals, polymer melt is extruded into filaments through a spinneret (not shown) of a melt spinning machine 10 and the filaments thus formed are fed into an air jet nozzle or ejector 12. The filaments are stretched pneumatically by compressed air jets as they pass through said air jet nozzle or ejector 12. Then, the filaments 20, ejected through the ejector 12, are deposited on a receiving conveyor 24 which advances said filaments at a fairly low speed compared with the above-mentioned ejection speed of the filaments. The conveyor 24 comprises an endless belt or a rotating drum which is composed of wire gauge, a perforated metal plate or the like. A pair of deflector plates 21 and 22 is provided above the conveyor 24. In addition, a suction box 25 is installed under the conveyor. By the construction mentioned above, the filaments being deposited on the conveyor are formed into a ribbon-shaped bundle 23 of a proper width wherein the filaments are moderately interconnected.

In the apparatuses as shown in FIGS. 2 and 3, a perforated rotating drum or rotor may be employed in place of the conveyor and also a bottomless box may be employed as the deflector. Preferably, the deflector is so arranged that the ejected filaments impinge on its wall or plate. Further, it is preferred that fluid jets are applied on to the ejected filaments at a certain angle with respect to their running down direction, before the ejected filaments impinge on the deflector plate(s), in order to increase the number of bends and loops of the filaments projecting from the sides of the ribbon-shaped bundle, and to enhance the entanglement of the filaments.

Thus, the ribbon-shaped bundle deposited on the conveyor is substantially free from twists and is composed of randomly oriented or arranged continuous filaments, each of which comprises random bends and loops along its length. More precisely, the filaments in the bundle are randomly bent and looped along their lengths and are randomly interconnected with each other. Further, the bent and looped ends protrude beyond the side ends of the bundle. From our study, it has been found that the width of the ribbon-shaped bundle is preferably in a range between 5 and 50 mm and the average diameter of the as-spun filaments is preferably less than 5 deniers, more preferably in a range from 0.3 to 3 deniers.

The ribbon-shaped bundle thus formed is then fed into a false-twisting zone wherein the bundle is false twisted and consolidated into a yarn.

Referring again to FIGS. 2 and 3, the ribbon-shaped bundle 23 is fed into a false-twisting zone through a nip between the conveyor 24 and an apron belt 33 and supplied to a false-twisting device 50. In the false-twisting zone defined between nip points 70 and 71, the ribbon-shaped bundle is false twisted by fluid torque jets which originate in the false-twisting device 50 and concurrently are consolidated into a yarn 80 of a substantially circular cross-sectioned fiber bundle. Then, the yarn is wound into a package by a winder 90 through a delivery roller means 60.

At the time when the ribbon-shaped bundle is false twisted, some of the continuous filaments are broken into discontinuous filaments of irregular lengths by the action of the fluid torque jets and/or by the friction

between the filament and the inner wall of the false-twisting device. Further, at the same time, the entanglement of the filaments is enhanced and some of both of the continuous and broken filaments are tightly wrapped around the fiber bundle. Thus, a yarn having a unique and novel configuration as mentioned hereinbefore can be obtained.

The false twisting is advantageously carried out by means of fluid torque jets in the form of compressed cold air, compressed hot air, super heated steam or the like. The fluid torque jets may be conveniently provided by a conventional false-twisting device, such as a fluid jet type twister. The apparatus whereby the process of this invention is advantageously carried out may further comprise a heater 40 and an oiling means 41, as shown in FIG. 2.

The configuration of the yarn of this invention may be controlled by adjusting the speed of the fluid jets in the ejector and/or in the false-twisting device, by varying the construction of a false-twisting device and/or by regulating the width of the ribbon-shaped bundle deposited on the conveyor, for example.

FIG. 4 illustrates an embodiment of the air jet nozzle or ejector which is useful in putting the process of this invention into practice. Compressed air is supplied into a chamber 11 from an inlet 13 and ejected as an air jet to an outlet 14 through a narrow area 15. As-spun filaments are fed into an inlet 16 and ejected from the outlet 14 with said air jets. Preferably, said ejector is installed at a proper distance from a spinneret.

FIG. 5 illustrates another embodiment of the air jet nozzle or ejector. An ejector of this type is preferably installed so that the spun filaments are introduced into the ejector without running down through open air. The ejector 17 is joined directly to a spinneret 18 attached to a spinning machine 10. Compressed air is supplied from an inlet 19 into a chamber 9 through holes 8 provided in the wall 17 of the chamber 9 and then ejected through an outlet 7 together with as-spun filaments extruded from the spinneret 18.

An embodiment of a false-twisting device of a fluid jet is shown in FIGS. 6 and 7, which is useful in practicing the process of this invention. Compressed air is provided from an inlet tube 51 and ejected into a tubular yarn passage 53 through a chamber 52 and fluid passages 54. The fluid passages 54 are perforated so as to direct the compressed air tangentially and angularly into the yarn passage 53. Two fluid passages 54 are shown in FIG. 7, but the number of the passage need not be limited to two. In FIG. 6, it is shown that the fluid passage 54 is provided at an angle of  $\theta$  with respect to the longitudinal axis (shown by a dotted line) of the tubular yarn passage 54. The angle of  $\theta$  is preferably in a range of  $30^\circ$  to  $60^\circ$ , more preferably in a range of  $35^\circ$  to  $45^\circ$ , in order to impart the desired ability to twist and aspirate the fibers being processed to the false-twisting device. Thus, fluid torque jets originate in the yarn passage of the false-twisting device and fibers are false twisted and consolidated into a yarn by the fluid torque jets as said fibers pass through the false-twisting device.

As the starting materials for manufacturing the yarn of this invention, fibers such as various types of synthetic fibers and blends of synthetic fibers and natural fibers can be used. However, synthetic organic fibers made of, for example, polyesters, polyamides and polyacrylates including copolymers thereof and novolac-

polyamide resins as well as blends of these polymers can be advantageously employed.

As will be appreciated, in the yarn of this invention, there may exist some discontinuous filaments having either a few or no folded ends. Further, the free ends of the broken filaments and bent and looped filaments protruding from the fiber bundle of the yarn provide desirable fuzzes on the surface of the yarn. It is preferable according to our experience that the ratio of broken ends in the fuzzes be more than 10 percent of all of the broken, bent and looped ends.

Advantages of this invention can be summarized as follows:

- a. the yarn of this invention has a spun yarn-like hand and appearance;
- b. the yarn of this invention is superior in bulkiness and uniformity of unwinding tension as compared with yarns of looped continuous filaments;
- c. the yarn of this invention shows a higher resistance to stretching as compared with wrapping yarns made of continuous filaments;
- d. spun-type yarns having desirable properties can be manufactured by a simple process without complicated steps as in the manufacturing of staple spun yarns;
- e. spun-type yarns having desirable properties can be manufactured with a high rate of efficiency and at a low-cost;
- f. as-spun filaments can be directly fed into the process of this invention, and;
- g. spun-type yarns can be manufactured from fine denier filaments and/or filaments having poor physical properties.

Further, the following methods may be applied to this invention;

- 1. to feed different kinds of fibers to ejector(s);
- 2. to extrude different kinds of polymers simultaneously from a single spinneret to form filaments and to feed them to ejector(s);
- 3. to make conjugated filaments and to feed them to ejector(s);
- 4. to melt or to eliminate the yarn partially before or after making a yarn, and;
- 5. to stretch and/or twist and/or twine the yarn of this invention.

The features of this invention will be more apparent by the following illustrative, but not limitative, examples, wherein an apparatus as shown in FIG. 3 was employed in practicing the process according to this invention.

#### EXAMPLE 1

Polyethylene terephthalate having an intrinsic viscosity of 0.55 was extruded through a spinneret. Filaments thus obtained were fed into an ejector, in which compressed air was supplied at  $1.25 \text{ kg/cm}^2 \text{ G}$ . The ejector was installed so that the spun filaments were introduced into the ejector without running down through the open air. The filaments were ejected with compressed air jets through a 3 mm diameter orifice at a speed of 6500 m/min. and simultaneously stretched pneumatically. Said filaments were deposited on a moving receiving conveyor after impinging on a pair of deflector plates to form a ribbon-shaped bundle having a width of 15 mm. The bundle was substantially free from true twists and consisted of randomly oriented, continuous filaments having random bends and loops. The bundle was then continuously fed to a false-twisting device in which compressed air was supplied at 3.5

kg/cm<sup>2</sup>G, false-twisted by fluid torque jets provided by the false-twisting device, at a speed of 263 m/min. and wound up as a consolidated yarn at a speed of 250 m/min. The yarn was of the configuration as shown in FIG. 1. In this yarn, some continuous filaments were broken into discontinuous fibers of irregular length. The yarn was of 50 metric count and both continuous filaments and discontinuous filaments emerging from the bundle were wrapped tightly around the bundle at various angles one above another. The bundle was composed of a blend of continuous filaments and broken filaments and was substantially free from twists.

A staple diagram of the obtained yarn is shown in FIG. 8. The values of parameters S and R were 2.7 and 0.034, respectively. Some of the properties of this yarn and these of a yarn spun by conventional ring spinning were measured and listed below in Table 1. The conventional spun yarn was composed of polyethylene terephthalate fibers having a length of 51 mm and a fineness of 2.5 deniers/fiber. As is shown in Table 1, the yarn of this invention is more bulky than the conventional ring spinning yarn and has a desirable distribution of the length of the bent, looped and broken ends. Furthermore, said yarn showed uniformity of unwinding tension when unwound from a cone in knitting due to the fact that the yarn does not have surface fibers longer than 10 mm.

Table 1

| metric count of the yarn (Nm)                          | Bulkiness of the yarn (cm <sup>3</sup> /gram) | The yarn of this invention |      |      | The conventional ring spinning yarn |     |      |
|--------------------------------------------------------|-----------------------------------------------|----------------------------|------|------|-------------------------------------|-----|------|
|                                                        |                                               | 1/50                       | 21.2 | 1/50 | 17.6                                |     |      |
| number of fuzes on the surface of the yarn (per meter) | kind of fuzes bent or looped end fiber end    | length of fuzes (mm)       | 3-6  | 6-10 | more than 10                        | 3-6 | 6-10 |
|                                                        |                                               |                            | 40   | 1    | 0                                   | 0   | 0    |
|                                                        |                                               |                            | 25   | 7    | 0                                   | 75  | 12   |

For the purpose of comparison, yarns composed of polyethylene terephthalate fibers were produced according to the methods described in British Pat. No. 1,102,095 and U.S. Pat. No. 3,079,746. The staple diagram of the yarn of British Pat. No. 1,102,095 is shown in FIG. 10 and that of the yarn of U.S. Pat. No. 3,079,746 is shown in FIG. 11. The former yarn had a parameter S value of 0.34 and a parameter R value of 0.2, while the latter yarn had a parameter S value of 0.04. Since the yarn of British Pat. No. 1,102,095 had multiple long loops on the yarn surface, the unwinding tension was not uniform and it was difficult to knit the yarn into fabric.

#### EXAMPLE 2

Polyethylene terephthalate having an intrinsic viscosity of 0.48 was extruded through a spinneret. Filaments thus obtained were fed into an ejector in which compressed air was supplied at 1.25 kg/cm<sup>2</sup>G, the ejector being installed so that the spun filaments were introduced into the ejector without running down through open air. The filaments were ejected with air jets through a 3 mm diameter orifice at a speed of 6500 m/min. and were simultaneously stretched pneumatically. Air jets provided by compressed air of 0.5 kg/cm<sup>2</sup>G were applied on to the ejected filaments be-

fore they impinged on the deflector plates. The filaments were then deposited on a moving receiving conveyor in the form of a ribbon-shaped bundle. The bundle was fed to the false-twisting device in which compressed air at 3.5 kg/cm<sup>2</sup>G was supplied, at a speed of 200 m/min. and was false-twisted by means of torque jets and then wound up as a consolidated yarn at a speed of 186 m/min. The yarn thus obtained was of 30 metric count and had a configuration similar to that of the yarn obtained in Example 1. The yarn had a spun-yarn-like hand and appearance. The staple diagram of this yarn is shown in FIG. 9. The values of parameters S and R were 2.1 and 0.007, respectively. The yarn was smoothly unwound from a cone and could be knitted easily.

#### EXAMPLE 3

The procedure in Example 2 was repeated, except that the speed of feeding a ribbon-shaped bundle to a false-twisting device was 300 m/min. and that the speed of winding the yarn was 290 m/min. The yarn thus obtained was of 47 metric count and the values of parameters S and R were 1.3 and 0.052, respectively. The yarn had a configuration similar to that of the yarn obtained in Example 1 and had a spun yarn-like hand and appearance.

#### EXAMPLE 4

Multifilaments made of nylon 6 (30 deniers, 12 filaments) free from oil treatment were fed into an ejector as shown in (FIG. 4) in which compressed air at 2 kg/cm<sup>2</sup>G was supplied. The ejected filaments were deposited on a receiving conveyor, which was moving at a speed of 200 m/min., in the form of a ribbon-shaped bundle and then said ribbon-shaped bundle was false-twisted by fluid torque jets and wound up at a speed of 200 m/min., as a consolidated yarn. When the bundle was false-twisted, some continuous filaments were broken into discontinuous fibers of irregular lengths. The yarn consisted of a core bundle bound together by and entangled with surface fibers emerging from said core bundle. The yarn was composed of both continuous and broken filaments having random bends and loops and core bundle was substantially free from true twists. The yarn was of 30 metric count and similar to the yarn obtained in Example 1, although the yarn had more radially projecting long loops than the yarn of Example 1. Some irregularity of unwinding tension was experienced in knitting this yarn into a fabric, but no actual trouble occurred. The values of parameters S and R of this yarn were 0.6 and 0.084, respectively.

## EXAMPLE 5

Polyethylene terephthalate having an intrinsic viscosity of 0.63 was extruded. Filaments thus obtained were stretched pneumatically by passing through an ejector (as shown in FIG. 4) in which compressed air at 3.5 kg/cm<sup>2</sup>G was supplied, and then deposited on a moving receiving conveyor through deflector plates in the form of a ribbon-shaped bundle. In this example, the ejector was installed at a distance of 40 cm from the spinneret. The ejected speed of the filaments was 6000 m/min. The ribbon-shaped bundle consisted randomly oriented, continuous filaments having random bends and loops. The ejected filaments had a fineness of 1.4 deniers, a tenacity of 2.8 g/denier, and an elongation of 35%. The bundle was false twisted and wound up at a speed of 150 m/min. to obtain a yarn. Some continuous filaments were broken in the false-twisting. The yarn had a tenacity of 193 grams, and an elongation of 40%. A yarn of 50 metric count was obtained. The configuration of the yarn was similar to that of the yarn obtained in Example 1 and the yarn had a spun-yarn-like hand and appearance. The values of parameters S and R were 1.8 and 0.05, respectively.

## EXAMPLE 6

Polyethylene terephthalate having an intrinsic viscosity of 0.58 was extruded and filaments thus obtained were stretched pneumatically when passing through an ejector (as shown in FIG. 4) which was installed at 40 cm from the spinneret. In the ejector, compressed air at 3.0 kg/cm<sup>2</sup>G was supplied. Ejected filaments were deposited on a moving receiving conveyor through deflector plates in the form of a ribbon-shaped bundle. The ejected speed of the filaments was 6100 m/min. The ribbon-shaped bundle consisted of folded, randomly oriented, continuous filaments of 0.3 denier per filament. The bundle was false twisted and wound up at a speed of 30 m/min. A yarn of 114 metric count was obtained and the configuration of the yarn was similar to that of the yarn obtained in Example 1. The values of parameters S and R were 2.1 and 0.02, respectively.

## EXAMPLE 7

As-spun bicomponent filaments which were composed of nylon-6 as one component and a copolymer of nylon 6 and nylon 66 as another component, were fed to the apparatus. The procedure employed was as described in Example 6, except that the ejecting speed of filaments was 3600 m/min., the fineness of filament was 1.1 deniers and the winding speed of the yarn was 100 m/min. Thus, a yarn of 38 metric count was obtained. The configuration of the yarn was similar to that of the yarn in Example 1. The value of parameter S was 1.2 and the value of parameter R was 0.087. When the yarn was heated at 150° C, crimps were present.

## EXAMPLE 8

Novolac resin (having an average molecular weight of 700) into which 20 percent by weight of nylon 6 was blended, was extruded into filaments and the filaments were provided to the apparatus. The procedure employed was as described in Example 6, with the exception that the ejecting speed of filaments was 4800 m/min., the distance between the spinneret and the inlet of the ejector was 60 cm and the fineness of filament was 1.1 deniers. The ejected filament had 0.6 g/denier of tenacity and 13% elongation. A 4.3 metric

count yarn was obtained with a configuration similar to that of the yarn in Example 1. The value of parameter S was 3.1 and the value of parameter R was 0.03. The yarn was cured in a mixture of sulfonic acid and folman. The cured yarn was nonflammable.

What we claim is:

1. A yarn consisting of a fiber bundle which is substantially free from true twists and composed of continuous and discontinuous filaments being complexly intertwined with one another and comprising random bends and loops along their lengths, said yarn having a value of a parameter S of not less than 0.5 and a value of a parameter R of not more than 0.1, said parameters S and R being defined as follows:

$$S = B/A$$

$$R = C/D$$

20 wherein A is the number of fibers contained in a test piece cut at a length of 10 mm along the yarn length under a load of 500 mg/denier and having lengths in the range of not less than 10 mm but less than 12 mm, B is the number of fibers contained in the test piece and having lengths in the range of not less than 12 mm but less than 30 mm, C is the number of fibers contained in the test piece and having lengths not less than 30 mm and D is the number of whole fibers contained in the test piece.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 990

ble to consolidate it into a yarn while some of said filaments are broken in the false twisting.

8. A process as claimed in claim 7, wherein continuous filaments are fed to a fluid jet nozzle or ejector and then deposited on a moving receiving conveyor to form said ribbon-shaped bundle.

9. A process as claimed in claim 8, wherein as-spun filaments are fed to said ejector whereon said filaments are stretched pneumatically by said fluid jet.

10. A process as claimed in claim 9, wherein said ejector is installed so that the as-spun filaments are introduced into said ejector without running down through open air.

11. A process as claimed in claim 8, wherein drawn filaments are fed to said ejector.

12. A process as claimed in claim 8, wherein the filaments ejected from said ejector impinge on the surface of a deflector installed above said moving receiving conveyor.

13. A process as claimed in claim 12, wherein fluid jet is applied to the ejected filaments before they impinge on the surface of said deflector.

14. A process as claimed in claim 7, wherein said ribbon-shaped bundle is false twisted by a fluid torque jet.

15. A process as claimed in claim 14, wherein some of said bundle composing filaments are broken into irregular lengths during the false twisting.

16. A process as claimed in claim 14, wherein some of said bundle composing filaments are partially and randomly wrapped around the bundle during the false twisting.

\* \* \* \* \*

20

25

30

35

40

45

50

55

60

65